

Nov. 24, 1936.

C. L. BEAL

2,061,749

RUBBER THREAD AND METHOD FOR MAKING THE SAME

Filed Oct. 11, 1933



## UNITED STATES PATENT OFFICE

2,061,749

RUBBER THREAD AND METHOD FOR  
MAKING THE SAMECarl L. Beal, Cuyahoga Falls, Ohio, assignor to  
American Anode, Inc., Akron, Ohio, a corpora-  
tion of Delaware

Application October 11, 1933, Serial No. 693,113

9 Claims. (Cl. 18—54)

This invention relates to elastic rubber thread such as that used for making stretchable fabrics for garments, etc. and relates especially to a novel method and apparatus for making from liquid rubber latex a substantially round rubber thread which will be admirably suited for weaving with textile threads to make elastic fabrics, and for other uses.

Heretofore, such rubber thread has been made commercially in one of two manners. In the older, and still more generally used method, a sheet of vulcanized calendered rubber is wrapped in several layers upon a large drum, the drum is caused to rotate and the sheet is cut into threads by means of a rotary knife mounted upon a lathe-like moving support. In a more recently devised method, liquid latex is extruded through a round nozzle into a coagulant and the extruded rubber filament is vulcanized to produce a smooth surfaced round rubber thread. Neither method is entirely satisfactory. The thread produced by the first described method has square cut corners which sometimes are irregular and tend to chafe easily when the thread is subjected to certain types of service and is further not well adapted for use in textile machinery designed to weave round textile threads. Although the advent of the smooth round extruded thread eliminated some of these disadvantages of square cut thread, it has not proved to be satisfactory in all respects. Thus, it has been found that the round extruded thread, when provided with a textile wrapping and woven together with textile threads to make an elastic fabric, will slip and fail to maintain its proper position or relationship in the woven structure, apparently because it is extremely smooth and presents few surface irregularities and consequently little frictional resistance to prevent slippage of the associated textile threads over its surface.

Accordingly, the objects of the present invention include the manufacture of a rubber thread possessing the weaving and processing advantages of round thread, which at the same time will not slip from its proper position when woven into a fabric; the manufacture of a substantially round rubber thread having slight surface irregularities adapted to increase frictional resistance of the thread without detracting from its resistance to chafing; the provision of a novel method of making from liquid latex a substantially round rubber thread; the provision of a method for forming a sheet of latex rubber and for cutting the sheet to produce a rounded

thread; the provision of rapid and economical means for producing from liquid latex large quantities of rounded thread; and other objects which will be apparent from the following description of the invention.

My invention, in a preferred embodiment, comprises forming from liquid rubber latex a continuous coherent sheet of rubber coagulum, and drying the sheet, if at all, to the extent only that the coagulum retains sufficient surface tack to cohere readily and remains in an easily deformable plastic state, but exhibits a substantial amount of resiliency, particularly in its outer or face portions, and then progressively subjecting the sheet to pressure applied at opposed points along parallel lines upon the two faces of the sheet to press opposite faces of the sheet along such lines into cohesive relationship and to deform the coagulum between such lines in such manner as to place at least one of the faces of the intervening portions of coagulum under considerable tension, then severing the sheet along the lines of cohesive engagement of the two faces, to form a plurality of strips of coagulum, which immediately upon severance of the sheet and consequent release of the restraining forces assume a substantially rounded cross-sectional configuration by reason of the deformation of the plastic coagulum effected by forces tending to equalize tension in the outer resilient portions of the deformed coagulum. I accomplish this procedure by forming from liquid latex a sheet of latex rubber coagulum, preferably containing fifty to seventy per cent. rubber (total solids) by weight and thirty to fifty per cent. water, such as a sheet formed from the concentrated latex of commerce without substantial loss of water, and then cutting the sheet, preferably after only slight surface drying, into a plurality of strips, with a device capable of cutting with a true shearing action simultaneously along a plurality of parallel lines. I have found that a rotary multiple disc shear in which the discs interlace slightly and have substantially right angular cutting edges is particularly well adapted to accomplish the deformation and severance of the plastic sheet to produce round strips. The manner in which this device operates upon the sheet of coagulum to accomplish this unexpected result will be set out in detail hereafter. At this point, it will suffice to say that in this manner I produce a substantially round or cylindrical rubber thread, the hemi-cylindrical surfaces of which originally were portions of opposite faces of the sheet of rubber coagulum, which faces,

in the thread, are effectually sealed or healed together by coherence of the rubber along approximately diametrically opposed longitudinal lines upon the thread surface. Along such lines 5 of jointure are slight surface irregularities resulting from the formation of the sealed joint, which add materially to the frictional resistance of the thread and prevent its slippage when woven with textile thread, but apparently do not 10 decrease chafing resistance as do the irregularities in prior square cut threads.

The invention will be more fully described with reference to the accompanying drawing, in which

Fig. 1 is a diagrammatic elevation of apparatus 15 adapted for carrying out the method of my invention.

Fig. 2 is a section taken on lines 2—2 of Fig. 1, illustrating more clearly the rotary multiple disc shear which is a part of the apparatus of Fig. 1.

20 Fig. 3 is a section taken on line 3—3 of Fig. 2.

Fig. 4 is an enlarged partial section taken on line 4—4 of Fig. 3, showing only a few of the disc shears and illustrating their action upon a sheet of rubber coagulum just as the discs come 25 into cutting relationship.

Fig. 5 is an enlarged partial section taken in the axial plane of the discs on line 5—5 of Fig. 3.

Figs. 6, 7 and 8 are sectioned perspective views 30 of short lengths of rubber threads produced by the present invention.

The preferred apparatus illustrated in the drawing comprises a hollow sheet metal deposition drum 10 rotatably mounted and provided with water pipe connections 11 for circulating 35 cooling water through the interior of the drum. The drum is rotated by means of a sprocket 12 and chain 13 deriving power from a source not shown. The lower portion of the drum dips into a body of latex 14 contained in a rectangular sheet metal tank 15 which is provided with a water jacket 16 through which cooling water may be circulated by means of pipe connections 17 and 18. Porous diaphragms 19 made of unglazed porcelain, asbestos, or similar material are inserted in the deposition tank near the surface 40 of the deposition drum and serve to separate the latex from the cathode liquid 20 which may be ordinary tap water, or a solution of a neutral conductive salt such as ammonium chloride or ammonium nitrate, surrounding metallic cathodes 21 which are inserted in both ends of the tank and are connected to the negative terminal 45 of a source of direct current (not shown). The positive terminal of the source of current is connected to a brush 22 which contacts with a slip ring 23 mounted on the drum shaft through which current may be conducted to the drum itself. The sides of the deposition drum are coated with an insulating paint or varnish, or 50 with a thin layer of rubber to insulate them from the latex, and the peripheral surface 24 of the drum preferably is made of zinc, cadmium, or similar metal capable of anodic solution without generation of gas. A stripping roller 25 of small 55 diameter is rotatably mounted with its surface almost in tangential contact with the surface 24 of the deposition drum 10 so that it may effectively strip a sheet of deposited rubber from the drum and deliver it to a conventional belt conveyor 26 arranged to convey the sheet to a multiple disc rotary shear 30.

The rotary shear comprises a bed plate 31, and two vertically slotted side frame members 32 connected at their upper extremities by tie bars 75 or plates 33. In the vertical slots in each of the

side frame members are fitted two boxes 34, the boxes being held in position vertically by adjusting screws 35 in each of the tie plates and over the top box. Journalled in the boxes are a pair of horizontally disposed arbors 36, the lower of which carries a driving sprocket 37 and a pinion 38 which meshes with a similar pinion 39 upon the upper arbor. Mounted upon each of the arbors are a number of hardened steel shear discs 40, which are separated by spacing rings or discs 41 of smaller diameter but of the same width as the shear discs 40, that width being substantially equal to the diameter of the thread or width of the strip to be made plus allowance for shrinkage of the rubber which occurs on drying. The shear discs 40 are of such diameter that, when they are mounted upon the arbors in the manner described, the disc peripheries will overlap or interlace slightly, to provide a true disc type shear. The shear discs 40, and spacing discs 41 are held 20 in place by pressing them against shoulders 42 at one end of each arbor by tightening threaded collars 43 at the opposite ends of the arbors. Two series of metal fingers 44 somewhat narrower than the shear discs are clamped upon supporting bars 45 so that the fingers extend into the spaces between the several shear discs at a position well past the cutting region of the shears, the function of these fingers being to aid in 25 removing cut strips from the spaces between the 30 shear discs.

Beyond the shearing apparatus is provided a pair of conventional endless belt conveyors 46 arranged one above the other in position to receive cut strips of rubber coagulum from the shearing device and to convey them horizontally through a tunnel dryer 47 heated as by hot air circulated through the dryer by means of ducts 48. If desired the dryer may be made sufficiently long, and heated to a temperature adequate to 40 vulcanize as well as to dry the coagulum. Under the delivery ends of the conveyors are provided boxes 49 into which the threads may fall preliminary to being wound or reeled upon bobbins 50.

When the apparatus is in operation, direct current flows through the brush 22 to the body of the deposition drum 10, through the zinc surface 24 to the body of latex 14, thence through the porous diaphragms, which are saturated with electro-conductive fluid, into the cathode liquid 20 and thence out through the cathodes 21. Under the influence of the current, the negatively charged particles of rubber and other solids suspended in the latex migrate toward and are deposited upon the peripheral surface of the 55 rotating deposition drum to form a continuous sheet 51 of water-containing latex rubber coagulum, preferably of a thickness approximately equal to the width of the disc shears, which sheet is continuously stripped from the drum after it 60 emerges from the body of the latex by means of the stripping roller 25, and is carried by the conveyor 26 to the multiple disc rotary shear 30.

The sheet of coagulum preferably is not heated or otherwise dried except for the slight natural surface drying which results from exposure to the atmosphere during the period after its emergence from the latex, but slight artificial drying during this period is not prohibited and in some cases may be desirable, particularly when conditions of operations are such that surface portions of the sheet are not sufficiently resilient to produce the desired effect upon shearing the rubber. The drying of the sheet however should not be carried further than is necessary to secure 70 75

the requisite surface resiliency and should never go so far as substantially to dry the sheet throughout its body. If slight forced surface drying is desired, a suitable heating chamber 5 may be provided about the conveyor 26.

The plastic and deformable but somewhat resilient and quite cohesive sheet of water-containing coagulum then is directed into the bight of the disc shears and as it progresses toward the 10 common axial plane of the discs, they apply a progressively increasing pressure to opposite faces of the sheet along longitudinal parallel lines. This pressure is concentrated at the points c (Fig. 4), in the sheet which pass along the 15 edges of the discs, because it is at these points that direct resistance to displacement of the sheet is offered by the cooperating edges of the adjacent interlacing discs and as a result thereof, the opposite faces of the sheet are in effect 20 pinched more and more closely together along the parallel lines determined by the several interlacing upper and lower discs. This pinching operation necessarily stretches the free faces f of the as yet unsevered intervening strips of co- 25 agulum and sets up substantially tensional forces in the surface portions thereof which, in obedience to well known physical laws, assume a rounded, practically semi-circular cross-sectional configuration. These surface tensional forces 30 are maintained and increased by the progressively pinching shears which press the opposite faces of the sheet closer and closer together with consequent progressively increased stretching 35 of the free faces of the coagulum until finally when the sheet reaches the cutting region of the shears and is severed along lines containing the points c, opposite faces of the sheet are, by the shearing action, brought into actual contact under high pressure and are pinched together. As 40 a result of this pinching and of the cohesive character of the coagulum, the formerly opposed faces of the sheet cohere along their severed edges so that upon release of the tensioning forces, which accompanies severance of the 45 sheet, the free faces of the now severed strips contact circumferentially under the internal tension, thereby circumferentially stretching the formerly unfree faces u of the strips and setting up tensional forces therein until the tension and 50 other forces throughout the strip are equalized. This equalization of the internal forces of the strip further deforms the still plastic coagulum and causes it to assume a substantially circular cross-sectional configuration as illustrated in Fig. 55 6. The equalization of internal forces and consequent shaping of the strip occurs immediately upon severance of the strip even though it is closely confined between the faces of the discs, because sufficient water—an excellent lubricant 60 for rubber—is expressed from the coagulum by the shearing operation to lubricate its surface thoroughly and to allow its easy movement along the sides of the shear discs. The several cut strips 52 of coagulum are separated by the shearing operation into upper and lower sets of alternating strips, which are directed respectively to the upper and lower conveyors to be dried and vulcanized in any suitable manner to produce finished rubber threads of substantially circular 65 cross section, each of which exhibits two substantially diametrically opposed longitudinal 70 seams 53 along the lines of cohesion of the opposite faces. The seams in most cases occur as continuous or discontinuous slightly projecting ribs as illustrated in Fig. 6, but in some instances 75

the seams open slightly to produce concave depressions 54 along the threads as in Fig. 7, although the effective cross-section of the thread remains substantially circular.

The invention has thus far been described as applied to the manufacture of round threads by shearing a sheet of coagulum substantially equal in thickness to the width of the shear discs, but it is by no means limited to such manufacture, and may be employed with equally satisfactory 10 results for making strips or bands of rubber. For example, if a sheet of coagulum is cut with a rotary disc shear in which the discs are considerably wider than the thickness of the sheet, a generally flat strip 55 having rounded edges of 15 substantially circular configuration will be produced. Diametrically opposed longitudinal seams 56 are evident along the approximate center of the rounded edges of such flat strips, just as in the round threads. It is apparent that 20 strips having oval, oblate spheroidal, and other rounded cross-sectional configurations may be produced by varying the width of the discs with relation to the thickness of the sheet of coagulum.

The many advantages of the present method 25 and its product are manifest. It provides for the efficient, rapid, and economical manufacture of a rubber thread which is particularly adapted for combining with textile threads or woven fabrics, but of course may be used in many other applica- 30 tions just as former types of elastic thread are used. It produces rounded threads such as are required for weaving, and at the same time provides sufficient surface irregularities in the thread to impart to it frictional resistance adequate to 35 prevent its slippage in a woven structure. The method is capable of continuous operation and is exceedingly well adapted for commercial production in that the apparatus required is compact, simple and relatively inexpensive. 40

It is obvious that many modifications and variations are possible in details of the above described procedure and apparatus. Thus, the sheet of rubber coagulum may be formed by coating a moving surface with a latex coagulant and 45 immersing the coagulant-coated surface into latex to deposit a sheet of rubber upon the surface, or a porous surface may be immersed in the latex to acquire a rubber deposit, or latex may be spread or flowed in sheet form on to a moving 50 surface, or other methods of forming a latex sheet possessing the requisite properties of resiliency, deformability and cohesiveness may be employed. Equivalent apparatus including other types of shears may be substituted for that shown 55 without departing from the scope of the invention.

Although I have illustrated the rubber thread produced by my invention as having an effective cross-section which is substantially circular, or in the case of flat bands, as having a circular 60 edge, it is to be understood that in practice, the actual cross-sections of the threads may vary somewhat from perfect geometric proportions and that the seams may not in all cases be exactly in diametric opposition. Accordingly, when I use 65 geometric terms in the specification and claims in describing the thread of this invention, it is to be understood that such terms are intended to include all such variations in proportions and are not intended necessarily to refer to exact geometrical configurations.

The term "latex" has been used in a generic sense to include all natural and artificial aqueous dispersions of rubber, gutta-percha, balata, and similar natural or synthetic gums, whether in the 75

unvulcanized, vulcanized, or reclaimed condition. The latex may be thickened, thinned, concentrated, diluted, vulcanized or otherwise preliminarily treated and may contain any desirable thickening, thinning, stabilizing, or other conditioning agents. Compounding ingredients such as vulcanizing agents, accelerators, age-resistors, fillers, pigments, softeners, etc. may be admixed with the latex as desired.

10 I claim:

1. A vulcanized rubber thread comprising an elongated strip of unmasticated latex rubber having the native colloidal structure of rubber deposited directly from liquid rubber latex, said strip having two opposed uncut faces and two opposed cut faces, the opposed cut faces exhibiting the characteristics of rubber faces cut by a shearing operation.

2. A vulcanized latex rubber thread having a cut edge and a line of surface irregularity extending longitudinally of the thread along the approximate mid-portion of the cut edge, said surface irregularity comprising a longitudinally extending reentrant groove serving to increase frictional resistance of the thread surface.

3. A vulcanized rubber strip having a cut edge and a seam extending longitudinally of the strip along the approximate mid-portion of the cut edge.

4. The method which comprises forming directly from liquid rubber latex a coherent sheet of latex rubber coagulum containing a substantial percentage of water distributed through the coagulum, progressively applying pressure to opposite faces of the sheet along a plurality of substantially opposed parallel lines upon the two faces of the sheet, and within the region of applied pressure simultaneously with the application of the pressure confining one face of each of the strips defined by said lines while leaving the opposite face of each of said strips unconfining, the adjoining faces of contiguous strips being alternately confined and unconfining, and severing the sheet along said lines.

5. The method which comprises forming directly from liquid rubber latex a coherent sheet of latex rubber coagulum containing a substantial percentage of water distributed through the coagulum, subjecting a plurality of parallel spaced zones of the sheet to progressive pressure applied from one side of the sheet substantially normally to the plane thereof and simultaneously subjecting the intervening zones to a like pressure applied from the other side of the sheet whereby ad-

jacent parallel zones are urged in opposite directions out of the normal plane of the sheet and the sheet is severed along the margins of said zones to produce strips of coagulum.

6. The method which comprises forming directly from liquid rubber latex a microporous sheet of cohesive and easily deformable but somewhat resilient rubber coagulum containing a substantial percentage of water distributed throughout its microporous structure, applying pressure to opposite faces of the sheet along a plurality of substantially opposed parallel lines upon the two faces of the sheet to press opposite faces of the sheet along said lines into cohesive relationship and to deform the coagulum between said lines in such manner as to place at least one of the faces of the intervening portions of coagulum under tension, and severing the sheet along the lines of cohesive engagement of the two faces, to produce strips of coagulum having substantially rounded severed edges, and drying the strips of coagulum.

7. The method which comprises forming directly from liquid rubber latex a microporous sheet of cohesive and easily deformable but somewhat resilient rubber coagulum containing a substantial percentage of water distributed throughout its microporous structure, and shearing the sheet of coagulum along a plurality of parallel lines to produce strips of rubber coagulum having substantially rounded edges, and drying the strips of coagulum.

8. The method which comprises forming directly from liquid rubber latex a sheet of water-containing rubber coagulum and drying the sheet to the extent only that the coagulum retains sufficient surface tack to cohere readily and remains in an easily deformable state, but exhibits a substantial amount of resiliency in its surface portions, and progressively shearing the sheet of coagulum along parallel lines to produce strips of rubber coagulum having substantially rounded edges, and drying the strips of coagulum.

9. The method which comprises electro-depositing rubber from liquid rubber latex upon a moving surface to form continuously a coherent sheet of water-containing coagulum, and while the sheet still contains a substantial part of the water which was deposited with the rubber from the latex, progressively shearing it simultaneously along a plurality of parallel lines of shear and drying the sheared strips to produce a plurality of rubber strips having rounded edges.

CARL L. BEAL.